

No. 723,212.

PATENTED MAR. 17, 1903.

P. A. KNAPPE.  
METHOD OF TREATING ORES.  
APPLICATION FILED AUG. 22, 1902.

NO MODEL.



Witnesses.

Ernest J. Emery  
John W. Johnson

Inventor.  
Paul A. Knappe  
by his Attorney, Frederick Emery -

# UNITED STATES PATENT OFFICE.

PAUL A. KNAPPE, OF GRANTVILLE, GEORGIA, ASSIGNOR TO AMERICAN AMALGAMATING COMPANY, OF BOSTON, MASSACHUSETTS, A CORPORATION OF GEORGIA.

## METHOD OF TREATING ORES.

SPECIFICATION forming part of Letters Patent No. 723,212, dated March 17, 1903.

Application filed August 22, 1902. Serial No. 120,623. (No specimens.)

To all whom it may concern:

Be it known that I, PAUL A. KNAPPE, a citizen of the United States, residing at Grantville, in the county of Coweta and State of Georgia, have invented an Improvement in Methods of Treating Ores, of which the following description, in connection with the accompanying drawing, is a specification, like letters on the drawing representing like parts.

My invention consists of an improved method of treating ore whereby I am enabled to extract the values efficiently and economically. Certain grades of ores, especially such as contain large percentages of sulfids, produce great quantities of slimes and are difficult to properly amalgamate on this account, a considerable amount of free precious metal being carried away by the slimes if a thorough amalgamation is attempted. By my process I am enabled to remove the greater portion of free precious metal from these ores by amalgamation without the usual difficulties and to separately recover the values from the concentrates and slimes.

My invention will be best understood from an illustration and description of one specific combination adapted to carry it into effect, while its scope will be particularly pointed out in the appended claims.

In the drawing I have shown in a vertical sectional view a combination of agitator and amalgamator, concentrating-table, and slime-tables so related as to be adapted to carry out my improved process.

In the drawing, A represents generally the primary receptacle for the crushed or pulverized ore and in which in the present instance I have combined the double function of agitator and amalgamator. The walls a, bottom b, and removable cover c of the receptacle are of any suitable material and the whole is supported upon a framework d. Within the receptacle A, I have shown means for gently agitating the pulp fed thereto, and for this purpose preferably employ the rotary upright agitator-arms e, carried by the radial supports f. Any means, however, for assisting the settling and the separation of the heavier particles from the lighter may be em-

ployed, and I am not limited to those disclosed, which are merely such as I prefer in practice. Supports f are fixedly attached to the hub-piece g, keyed or otherwise suitably fastened to the vertical shaft h to rotate therewith. A slow rotation is imparted to the shaft h and the attached agitating-arms through the bevel-gears i and the pulleys j.

At k is provided a feed-inlet for the pulp. A series of slime-discharge outlets l l' is shown on the opposite side of the agitator below the level of the feed-inlet. To illustrate my process, I have here shown but two such outlets, the upper one, l, for the removal of the finer slimes, and the lower one, l', for the medium slimes; but it is evident that this series may be indefinitely extended as conditions may require. Each slime-outlet is connected through its respective discharge-pipe m m', under the control of valves n n', with its separate slime-table L L', which may be of any of the well-known forms of construction, but which I have shown diagrammatically only, inasmuch as the specific construction is immaterial to my process.

The bottom b of the agitator A is corrugated or grooved or otherwise suitably indented to afford pockets o for the retention of free mercury and the amalgam resulting from the union thereof with the precious metal in the pulp.

A heavy-materials outlet p is provided in the walls of the agitator for the discharge of the concentrates and other heavy particles. This discharge is located slightly above the mercury-space in the bottom to avoid drawing any of the mercury or amalgam therefrom and is connected through discharge-pipe q, controlled by the valve r, with the receiving-compartment of the concentrating-table P. The latter may be of any suitable construction and I have shown the same in a conventional manner only.

A valve-controlled outlet s at the bottom of the agitator affords means for removing at the necessary intervals the accumulated mercury and amalgam, together with such heavy particles as are unsuceptible to amalgamation.

My process, which is preferably continu-

ous, is carried out in the following manner: The ore is pulverized to the mesh necessary to liberate the mineral from the gangue by either the wet or dry process. The ore so 5 crushed is continuously fed into the receptacle A, the necessary amount of water being added, either before or after it reaches the receptacle, to form a pulp of the proper consistency and permit a ready separation of the 10 heavier particles from the lighter and the gravitation or settling of the same to the bottom of the receptacle. The circulation of the mass, which is maintained by the gentle movement of the upright fingers, accelerates and 15 aids the natural gravitation of heavier particles and separates or classifies the pulp particles into layers according to their density. The lighter particles near the surface of the settler form the slimes, and these are with- 20 drawn continuously through the discharge-pipes placed at different levels and corresponding to their respective classes or layers, the finest slimes being discharged through the uppermost outlet, the coarsest through the 25 lowest slime-outlet, and the intermediate slimes through their respective intermediate outlets. The heaviest particles and concentrates, together with the particles of free metal, respond to the laws of gravity and settle to 30 the bottom of the receptacle, where they come in contact with the free mercury contained therein, which latter forms an amalgam with such amalgamatable metals as are among them and is withdrawn as often as desired 35 through the discharge-pipe s. Additional mercury is fed into the receptacle to the extent necessary to replace the withdrawn amalgam. The discharge-pipe for the heavy mineral or pulp is located somewhat above 40 the mercury-level and within the area of agitation, so that there is always a bed of mineral or concentrates in the lower part of the agitator kept in motion by the agitator-arms. The circulation or movement of these heavier 45 particles over and about the bottom of the settler removes the amalgamatable metal from the mass. The surplus concentrates and minerals are removed through the heavy- materials discharge p as rapidly as fresh ad- 50 ditional particles are added to the mass through the settling process. The heavy materials or concentrates which are drawn from the lower part of the agitator are conveyed to the concentrating-table and concentrated in 55 the usual way and are then again subjected to amalgamation by any of the methods in use— plate, pan, barrel, or tube. The material which is taken to the concentrating-table contains in addition to the sulfids some free gold 60 which did not come in contact with the mer- 65 cury in the agitating-receptacle and also some amalgam escaped from the pockets. This gold and amalgam are concentrated with the sulfids and passing off the table are recovered when the mixture is again subjected to amalgamation. The different grades of slimes are 65 delivered to the slime-tables or other suitable

devices for concentrating or separating the fine mineral from the worthless material, the slime-concentrates secured in this manner being treated by amalgamation, cyanid, or other process of recovery suitable to the particular kind of ore under treatment. The values in the slimes are largely represented by minute particles of lead, zinc, copper, iron, and sulfids of their metals carrying gold, and by an economical concentration these slimes may be made valuable. 7c

By the employment of my invention I am enabled to maintain a continuous process and avoid the delays and much expense heretofore incidental to the recovery of values from ores containing large percentages of sulfids. I am also enabled to successfully and continuously treat sulfid ores crushed by the 85 dry process, which has heretofore been difficult, particularly in methods employing plate amalgamation, owing to the impossibility of maintaining a pulp of the proper consistency. 90

It is to be understood that my method may be carried out in a great variety of ways and is in no way limited to the specific apparatus disclosed, which is submitted for illustrative purposes only. 95

I claim—

1. The process of treating ores which consists in continuously feeding pulp to a settler and grading the same therein, continuously withdrawing each of the lighter strata before contact with mercury, causing mixing contact of the heaviest pulp particles with mercury, discharging the non-amalgamable portion thereof, and separately recovering the values from the different grades withdrawn from the settler. 100 105

2. The process of treating ores which consists in continuously feeding pulp to a settler and gently agitating the same therein to cause separation of the lighter from the heavier particles and a grading of the same, causing mixing contact of the heaviest pulp particles with mercury, continuously withdrawing each of the superimposed lighter strata before contact with mercury and separately recovering the values therefrom. 110 115

3. The process of treating ores which consists in continuously feeding pulp to a settler and gently agitating the same therein to cause separation of the lighter from the heavier particles and a grading of the same, causing mixing contact of the heaviest pulp particles with mercury, withdrawing the non-amalgamable portion thereof and concentrating the same, continuously withdrawing each of the superimposed lighter strata before contact with mercury and separately recovering the values therefrom. 120 125

In testimony whereof I have signed my name to this specification in the presence of two subscribing witnesses.

PAUL A. KNAPPE.

Witnesses:

THOS. L. WOOD,  
E. S. BROOKS.